# EUROPEAN PATENT APPLICATION

(11) **EP 1 847 623 A1**
(43) Date of publication of application: **24.10.2007**
(21) Application number: 06119981.6
(22) Date of filing: 01.09.2006
(51) Int. Cl.: C21D 9/00, C21D 1/52

(54) **Method for heating a metal material**

(30) Priority: 11.04.2006 SE 0600813
(71) Applicant: AGA AB, 181 81 Lidingö (SE)
(72) Inventor: Eichler, Rudiger, 187 41 Täby (SE)
(74) Representative: Örtenblad, Bertil Tore

(57) **Abstract**

The invention is characterized in that the heating power of the flame (10) of the DFI burner (1) is pulsated in cycles, so that the heating power is alternated between at least two different, predetermined powers, where each predetermined power, respectively, is maintained during a certain predetermined time period, where some powers are made to be lower than others, in that the powers are made to be low enough, and the time periods are made to be short enough, so that the combination of the powers and their corresponding time periods results in that the surface of the metal slab (3) is not heated above a certain, predetermined limit temperature during the time periods of the higher powers, in that this pulsating heating of the metal material (3) is interrupted when a certain stop condition is fulfilled, and in that the metal material (3) thereafter is heated to another predetermined, final, homogenous temperature by the use of another, conventional heating method.

## Description

The present invention relates to heating of metal materials, such as metal blanks, parts, etc., using a DFI (Direct Flame Impingement) burner.

DFI burners are used for heating various metal materials. Instead of heating a volume of the interior of for example an industrial furnace, and hence indirectly heating a material, the flame is impinged directly upon the surface of the material, thus heating it directly. This gives rise to better heat transfer efficiency from the burner to the material.

A common type of DFI burner is the so called oxyfuel type DFI burner, which is a burner in which the oxidant has higher oxygen content and lower nitrogen content as compared to air.

When heating using a DFI burner, the temperature of the surface of the metal material increases very quickly, and unwanted effects, such as melting, can occur if the heating is allowed to progress during too long a time within the same area of the surface of the metal material. Today, therefore, DFI burners are primarily used for heating of metal parts of relatively small cross sections, such as wires, sheets and smaller billets. As for these metal parts, the temperature throughout the material will have time to reach a sufficient level before the surface of the material deteriorates as a consequence of the intensive heat.

In some cases, these materials are conveyed through the flames of DFI burners. In case of a stoppage of production, the DFI burners may have to be shut down in order to prevent the surfaces of the materials from deteriorating.

It would be desirable if the higher efficiency of heat transfer when using DFI burners could be used also when heating slabs of larger cross sections. However, this is not possible using the known art. Namely, there is not enough time for such slabs to be sufficiently heated throughout the whole volume of the material before the surface of the material deteriorates, for example by melting.

The present invention solves the above described problem.

Thus, the present invention relates to a method for heating metal materials, such as a slab or a billet, using at least one DFI burner, and is characterized in that the heating power of the flame of the DFI burner is pulsated in cycles, so that the heating power is alternated between at least two different, predetermined powers, where each predetermined power, respectively, is maintained during a certain predetermined time period, where some powers are made to be lower than others, in that the powers are made to be low enough, and the time periods are made to be short enough, so that the combination of the powers and their corresponding time periods results in that the surface of the metal slab is not heated above a certain, predetermined limit temperature during the time periods of the higher powers, in that this pulsating heating of the metal material is interrupted when a certain stop condition is fulfilled, and in that the metal material thereafter is heated to another predetermined, final, homogenous temperature by the use of another, conventional heating method.

In the following, the invention will be explained in detail, with reference to an embodiment described in the accompanying drawings, wherein:
Fig. 1 is an overview of a DFI burner which is made to heat a metal material in the form of a slab according to the method of the present invention.

Fig. 2 is a diagram showing the power, as a function of time, for the DFI burner in Fig. 1, according to the method of the present invention.

Fig. 1 shows an oxyfuel type DFI burner 1, which is arranged in the interior of an industrial furnace 2, in such a way so that its flame 10 is made to impinge directly upon a metal material 3 in the form of a slab, also arranged in the interior of the furnace 2. The metal material 3 is large enough for a heating of the whole volume of the metal material 3 up to a certain desired, predetermined temperature profile using the DFI burner 1 continuously, would lead to deterioration of the surface of the metal material 3, for example by melting. Preferably, the metal material is in the form of a slab having a weight of between 10 and 160 tons.

The DFI burner 1 is provided with a supply inlet for fuel 4 and a supply inlet for oxidant 5. The fuel could be any suitable fuel, such as for example a gaseous fuel such as natural gas, a liquid fuel such as oil, or a solid fuel such as pulverized coal. The oxidant could be any suitable, gaseous oxidant. According to a preferred embodiment, the oxygen content of the oxidant is at least 85% by weight.

The supply inlets 4, 5 are connected to a control unit 6, which is made to continuously control the supply of fuel and oxidant. The control unit 6 is also connected to a temperature sensor 7, arranged in the interior of the furnace.

The temperature sensor 7 is arranged to pyrometrically measure the temperature of the part of the surface of the metal material 3 being impinged by the flame 10 of the DFI burner. The measured value for this surface temperature is continuously transmitted to the control unit 6.

The control unit 6 is thus arranged to control the heating power of the DFI burner 1, through the control of the amount of fuel and oxidant, respectively, being supplied to the DFI burner 1 at any given moment in time through the supply inlets 4, 5. This control takes place in the present embodiment by the simultaneous, proportional increase or decrease of both the amount of fuel and the amount of oxidant.

In the present embodiment, the control is carried out such that the heating power of the DFI burner 1 alternates between two different states; one state with a higher power and one state with a lower power. The lower power can, in effect, be zero. In other words, the DFI burner 1 can be switched off when the lower power prevails, and it is reignited when the higher power commences. However, it is possible to use more than two different, alternating power states, and that these power states each are associated with any suitable power value between zero and the maximum power of the DFI burner. For example, it is possible that a lower power state is such that only a flame of a pilot type is burning, so that the burner 1 does not need to be reignited when leaving the lower power state.

In the following, the term "turned on state" denotes the higher power state of the present embodiment, and the term "turned off state" denotes the lower power state in the present embodiment. A method alternating between at least one turned on state and at least one turned off state is herein denoted by the term "on/off operation".

Each power state is associated with a corresponding time period. Thus, the control unit 6 is made to control the supply of fuel and oxidant, respectively, to the DFI burner 1, so that the turned on state is made to prevail during a certain first time period, after which the turned off state is made to prevail during a certain second time period, after which the turned on state is made to prevail during the first time period again, and so on, in an alternating manner.

During the first time period, the metal material 3 is heated. Had the turned on state been maintained during a longer time, the surface of the metal material 3 had finally deteriorated, as a consequence of the too elevated temperature. However, the turned off state is commenced before such a damage occurs.

In the following, the control of the power of the DFI burner 1 over time in the present embodiment will be explained in greater detail, with reference to Fig. 2, showing a schematic diagram over the emitted power of the DFI burner 1 as a function of time from the beginning of the operation.

At the start of the heating operation, the metal material 3 maintains a certain known, homogenous temperature, for example 600°C. To start with, the power of the turned on state is made to be the full power of the DFI burner. The length of the second time period is made to be long enough, as compared to the length of the first time period, in order for the surface of the metal material 3 to cool down enough, by means of heat being conducted down into the material during the turned off state, not to be heated above a certain predetermined, maximal surface temperature during the next time period of a turned on state. This maximal surface temperature is herein denoted by the term "limit temperature".

The limit temperature is, for example, set so that it is just below the temperature desired to be the final temperature throughout the whole volume of the metal material 3. If, for example, a slab is to be heated to 1 225°C, the limit temperature is set to 1 225°C - X°C, where X, by way of example, is 100, or another suitable security margin. However, the limit temperature can be set to any other temperature suitable for the specific purposes of the procedure according to the present invention, such as just below the melting point of the metal material 3, or just below the melting point of the oxide scale of the metal material 3.

Initially, the lengths of both of the time periods can be set based upon an empirical investigation using the same type of metal material 3 which will be heated, the used industrial furnace 2, the initial temperature of the metal material 3, etc. The lengths of the initial time periods can also be dynamical, in the sense that their respective power states are maintained up until the point where a certain condition is fulfilled.

Thus, the surface of the metal material 3 is heated during the turned on state. During the turned off state, the heat is conducted from surface of the metal material 3 down into the interior parts of the metal material 3, and is thus made to heat the rest of the volume of the metal material 3 via thermal conduction, at the same time as the surface layer of the metal material 3 cools down. For each alternating cycle between the turned on state and the turned off state, the volume of the metal material 3 is further increasingly heated, whereby the average temperature, over a complete cycle, of its surface layer consequently also increases.

This initial, alternating process is shown graphically in Fig. 2 as "Phase A". Exemplifying values during Phase A is 15 seconds for the first time period (turned on state), and 15 seconds for the second time period (turned off state).

The control unit 6 is made to continuously obtain information on the average surface temperature of the metal material 3, from the temperature sensor 7. As the average surface temperature surpasses a certain first, predetermined value, the control unit 6 is made to shift modes, so that the time period of the turned on state is shortened in each alternating cycle. This is denoted in Fig. 2 as "Phase B". This shortening of the time period of the turned on state will result in the surface of the metal material 3 being less heated during every first time period, during which the turned off state prevails, and its temperature does not manage to reach the predetermined limit temperature during the turned on state, albeit the higher interior temperature of the metal material 3 relative to the initial temperature, as compared to during the beginning of Phase A.

As the average surface temperature surpasses a certain second value, the control unit 6 is made to shift modes, so that, additionally, the time period of the turned off state is extended in each alternating cycle. This is denoted in Fig. 2 as "Phase C". This elongation of the time period of the turned off state results in that the surface of the metal material 3 can cool down to a greater extent, as compared to during Phase B, during the turned off state, in order to guarantee that the surface of the metal material 3 still does not surpass the predetermined limit temperature in the following.

As the average surface temperature surpasses a certain third determined value, the control unit 6 is made to shift modes, so that the power of the turned on state is reduced, for example to half of the maximum power of the DFI burner, which further reduces the heating during the turned on state. This is denoted in Fig. 2 as "Phase D".

Phase D is maintained, with its moderate heating power, until the average surface temperature of the metal material 3 reaches a certain predetermined value. Alternatively, Phase D is maintained during a certain predetermined time period. The predetermined, average surface temperature or the predetermined time period can be empirically determined, based on the material being heated, the desired final, homogenous temperature, etc.

In order to reach a predetermined, final, homogenous temperature in the entire volume of the metal material 3, another heating method is subsequently used, for example using a furnace with a conventional burner, to finish the heating of the metal material 3. For example, if the desired, final, homogenous temperature is 1 225°C, this secondary heating step is maintained until this temperature has been reached throughout the entire volume of the metal material 3.

Thus, in the process described above, with reference to Phase A, Phase B, Phase C, and Phase D, the corresponding power values and/or the corresponding time periods over successive cycles are changed, so that the higher power value is reduced, the time period corresponding to the lower power value is lengthened and/or the time period corresponding to the higher power value is shortened, so that the average power impinged upon the surface of the metal material 3 during a subsequent cycle is less than the average power during a previous cycle.

However, the control unit 6 is not limited to performing a control such as the one described in conjunction with the phases A, B, C, and D. Rather, any suitable control can be used, where the power values and/or their corresponding time periods are changed over successive cycles, so that higher and/or lower power values are reduced, time periods corresponding to lower power values are lengthened and/or time periods corresponding to higher power values are shortened, so that the average power impinged upon the surface of the metal material 3 during a subsequent cycle is less than the average power during a previous cycle.

In the described embodiment, power values and/or their corresponding time periods are changed as a function of the instantaneous surface temperature of the metal material 3.

However, the control can be carried out based not only on the instantaneous surface temperature of the metal material 3, which is read off by a pyrometer, but also on other parameters, such as, for example, calculations and/or values based on experience. Also, another type of temperature sensor can be used instead of a pyrometer, such as, for example, a thermocamera.

Also, the present method can be used as a complement to other heating methods, for example in an industrial furnace, together with other heating apparatus. One example of this is the use in a car-type furnace, for the heating of a bloom, in which case the furnace is heated using its proper, conventional heating elements or burners. In this case, additional burners are positioned for heating according to the method of the invention, for example in the arc or in the lower part of the furnace, pointed directly at the bloom. The slabs are charged cold or preheated.

Above, various preferred embodiments have been described. However, it will be apparent to those skilled in the art that many modifications can be done to the described embodiment, without departing from the idea of the invention. Thus, the invention shall not be limited by the described embodiments, but rather be variable within the scope of the enclosed claims.

## Claims

1. Method for heating metal materials, such as a slab or a billet (3), using at least one DFI burner (1), **characterized in that** the heating power of the flame (10) of the DFI burner (1) is pulsated in cycles, so that the heating power is alternated between at least two different, predetermined powers, where each predetermined power, respectively, is maintained during a certain predetermined time period, where some powers are made to be lower than others, **in that** the powers are made to be low enough, and the time periods are made to be short enough, so that the combination of the powers and their corresponding time periods results **in that** the surface of the metal slab (3) is not heated above a certain, predetermined limit temperature during the time periods of the higher powers, **in that** this pulsating heating of the metal material (3) is interrupted when a certain stop condition is fulfilled, and **in that** the metal material (3) thereafter is heated to another predetermined, final, homogenous temperature by the use of another, conventional heating method.

2. Method according to claim 1, **characterized in that** the stop condition consists **in that** the average temperature of the surface of the metal material (3), over a complete cycle, surpasses a certain predetermined value.

3. Method according to claim 1, **characterized in that** the stop condition consists **in that** a certain time has gone by from the start of the process.

4. Method according to any of the preceding claims, **characterized in that** the different predetermined power values are obtained through control of the amount of supplied fuel and oxidant to the DFI burner (1).

5. Method according to any of the preceding claims, **characterized in that** the control of the DFI burner (1) is carried out by the use of an on/off operation.

6. Method according to any of the preceding claims, **characterized in that** the limit temperature is lower than the melting point of the metal material (3).

7. Method according to any of the claims 1 - 5, **characterized in that** the limit temperature is lower than the melting point of the oxide scale of the metal material (3).

8. Method according to any of the claims 1 - 5, **characterized in that** the limit temperature is lower than the final, homogenous temperature of the metal material (3).

9. Method according to any of the preceding claims, **characterized in that** the corresponding power values and/or the corresponding time periods over successive cycles are changed, so that higher and/or lower power values are reduced, time periods corresponding to lower power values are lengthened and/or time periods corresponding to higher power values are shortened, so that the average power impinged upon the surface of the metal material (3) over a subsequent cycle is less than this average power over a previous cycle.

10. Method according to claim 9, **characterized in that** that power values and/or their corresponding time periods are changed as a function of the instantaneous surface temperature of the metal material (3).

11. Method according to any of the preceding claims, **characterized in that** the said oxidant has an oxygen content of more than 85% by weight.

12. Method according to any of the preceding claims, **characterized in that** the DFI burner (1) is used in an industrial furnace (2) in cooperation with other heating apparatus.
